

1

2,833,714

## LUBRICANT COMPOSITIONS

Eugene E. Richardson, Hammond, and Roger W. Watson, Highland, Ind., assignors to Standard Oil Company, Chicago, Ill., a corporation of Indiana

No Drawing. Application September 28, 1955  
Serial No. 537,268

6 Claims. (Cl. 252—32.7)

This invention pertains to improved lubricant compositions and more particularly pertains to internal combustion engine lubricant compositions which inhibit cam follower pitting and/or wear and which inhibit the sticking of hydraulic valve-lifters.

Many modern automobile engines are designed with hydraulic valve-lifters for smoother and more efficient engine operation. In the operation of hydraulic valve-lifters, the lifters ride on the cam shaft converting the rotary motion of the cam into a reciprocating motion, which in turn opens and closes the valves. The bottom of the valve-lifter is known as the cam follower. The hydraulic part of the valve-lifter functions by means of a plunger on the inside of the valve lifter barrel, together with a ball-check and a spring. To obtain higher efficiency and greater horsepower, larger valves, high valve spring pressures and camshafts which produce more rapid valve opening and closing are employed. In the operation of such engines, greatly increased pressures are encountered where the camshaft lobes come into contact with the faces of the valve-lifters resulting in excessive and severe cam and lifter wear as well as pitting of the cam followers. This wear and/or pitting cannot be adequately inhibited by most present-day internal combustion engine crank-case lubricants. Surprisingly, the type of anti-wear properties which will inhibit piston ring and/or cylinder wear are not necessarily the same as the anti-wear properties necessary to prevent cam and lifter wear and/or pitting; hence many lubricants which are effective in inhibiting ring and cylinder wear are ineffective in preventing cam and lifter wear. A further complicating factor in this problem is caused by the materials used in making the camshaft and valve-lifters since different metals and metal combinations are used for this purpose in the various engines. Camshaft and valve-lifter combinations of different metals create different requirements on the lubricant in that certain types of anti-wear additives may be effective with some cam-lifter metal combinations but ineffective with other metal combinations. Furthermore, because of the small clearances between the plunger and the barrel of hydraulic valve-lifters, extremely small amounts of deposits such as varnish and/or rusting may cause sticking of the valve-lifter. Hence, it is essential for good engine operation to provide a lubricant which will, in addition to inhibiting wear and/or pitting, also inhibit the formation of varnish and/or rusting in the valve-lifter.

It is an object of this invention to provide a lubricant composition which will not cause sticking of hydraulic valve-lifters and which will inhibit cam follower wear and/or pitting. Another object of the invention is to provide a crank-case lubricant which will be substantially free of any tendency to cause valve-lifter sticking and/or rusting and which will have cam follower anti-pitting and anti-wear properties. Another object of the invention is to provide an improved lubricant for internal combustion engines. Still another object of the invention is to

2

provide a method of preventing the sticking of hydraulic valve-lifters and the pitting and/or wear of cam followers in internal combustion engines. Other objects and advantages of the invention will become apparent from the following description thereof.

In accordance with the herein described invention, the above objects can be attained by incorporating in a viscous oil, i. e., an oil having a Saybolt Universal viscosity above about 80 seconds at 100° F., containing 10 about 0.002 and 10% of a phosphorus- and sulfur-containing detergent-type lubricating oil additive, between about 0.001 and 5% of the polymerization products of unsaturated fatty acids such as linoleic acid, and between about 0.001 and 5% of stearic acid or its salts. The 15 polymerization products may have a molecular weight between about 400 and 2000.

The detergent-type lubricating oil additive used is one which contains phosphorus and sulfur. The function of this type of additive is to inhibit the formation of sludge 20 and/or varnish-like products which are deposited in the engine and/or about the valves and rings of the engine. Detergent additives of this type are usually used in amounts of from about 0.002 to about 10%, and preferably from about 0.01% to about 5%. Among the 25 phosphorus- and sulfur-containing addition agents are the neutralized reaction products of a phosphorus sulfide and a hydrocarbon, an alcohol, a ketone, an amine or an ester. Of the phosphorus sulfide reaction product additives, the neutralized reaction products of a phosphorus sulfide, such as a phosphorus penta-sulfide, and a hydrocarbon (note U. S. 2,316,082) are preferred.

The preferred hydrocarbon used for reaction with the phosphorus sulfide is a mono-olefin hydrocarbon polymer resulting from the polymerization of low molecular 35 weight mono-olefin hydrocarbons, such as propylene, butenes, amylanes or copolymers thereof. Such polymers may be obtained by the polymerization of mono-olefins of less than 6 carbon atoms in the presence of a catalyst, such as sulfuric acid, phosphoric acid, boron fluoride, 40 aluminum chloride or other similar halide catalysts of the Friedel-Crafts type.

The polymers employed are preferably mono-olefin polymers or mixtures of mono-olefin polymers and iso-mono-olefin polymers having molecular weights ranging 45 from about 150 to about 50,000 or more, and preferably from about 500 to about 10,000. Such polymers can be obtained, for example, by the polymerization in the liquid phase of a hydrocarbon mixture containing mono- and isomonoolefins, such as butylene and isobutylene at 50 a temperature of from about —80° F. to about 100° F. in the presence of a metal halide catalyst of the Friedel-Crafts type, such as for example, boron fluoride, aluminum chloride, and the like. In the preparation of these 55 polymers, a hydrocarbon mixture containing isobutylene, butylenes and butanes recovered from petroleum gases, especially those gases produced in the cracking of petroleum oils in the manufacture of gasoline can be used.

Another suitable polymer is that obtained by polymerizing a mixture of propene with other close-boiling saturated hydrocarbons. An aluminum chloride-iso-octane complex may be used as the catalyst at a temperature of about 50 to 100° F. to produce the polymer which may then be fractionated to a molecular weight, preferably from about 500 to 1000 or higher.

Paraffinic hydrocarbons such as bright stock residuums, lubricating oil distillates, waxes, and the like can be reacted with phosphorus sulfide. Olefins having 16 to 30 carbon atoms or higher may be reacted with the phosphorus sulfide. Other hydrocarbons that can be reacted with a phosphorus sulfide are aromatic hydrocarbons such as benzene, naphthalene, diphenyl, alkylated aromatic hy-

drocarbons such as benzene having alkyl substituents containing preferably at least 8 carbon atoms and the like.

The phosphorus sulfide-hydrocarbon reaction product can be readily obtained by reacting a phosphorus sulfide, for example  $P_2S_5$  with the hydrocarbon at a temperature of from about 200° F. to about 500° F., and preferably from about 200° F. to about 400° F., using from about 1% to about 50%, and preferably from about 5% to about 25% of the phosphorus sulfide in the reaction. It is advantageous to maintain a non-oxidizing atmosphere, such as for example, an atmosphere of nitrogen above the reaction mixture. Usually, it is preferable to use an amount of the phosphorus sulfide that will completely react with the hydrocarbon so that no further purification becomes necessary; however, an excess amount of phosphorus sulfide can be used and separated from the product by filtration or by dilution with a hydrocarbon solvent, such as hexane, filtering and subsequently removing the solvent by suitable means, such as by distillation. If desired, the reaction product can be further treated with steam at an elevated temperature of from about 100° F. to about 600° F.

The phosphorus sulfide-hydrocarbon reaction product normally shows a titratable acidity which is neutralized by treatment with a basic reagent. The term "neutralized reaction product of a phosphorus sulfide and a hydrocarbon" as used herein means a phosphorus sulfide-hydrocarbon reaction product having at least 1% of its titratable acidity neutralized by the reaction with a basic reagent. The phosphorus sulfide-hydrocarbon reaction product when neutralized with a basic reagent containing a metal constituent is characterized by the presence or retention of the metal constituent of the basic reagent. Prior to neutralization the reaction product can be hydrolyzed and clayed to remove inorganic acids of phosphorus as described in U. S. 2,688,612 issued to R. W. Watson September 7, 1954.

The neutralized phosphorus sulfide-hydrocarbon reaction product can be obtained by treating the acidic reaction product with a suitable basic compound, such as hydroxide, carbonate oxide or sulfide of an alkaline earth metal or an alkali metal, such as for example, potassium hydroxide, sodium hydroxide, sodium sulfide, calcium oxide, lime, barium hydroxide, barium oxide, etc. Other basic reagents can be used, such as for example, ammonia or an alkyl or aryl-substituted ammonia, such as amines. The neutralization of the phosphorus sulfide-hydrocarbon reaction product is carried out preferably in a non-oxidizing atmosphere by contacting the acidic reaction product either as such or dissolved in a suitable solvent, such as naphtha with a solution of the basic agent. As an alternative method the reaction product can be treated with solid alkaline compounds such as KOH, NaOH,  $Na_2CO_3$ , CaO, BaO,  $Ba(OH)_2$ ,  $Na_2S$ , and the like, at an elevated temperature of from about 100° F. to about 600° F. Neutralized reaction products containing a heavy metal constituent, such as for example, tin, titanium, aluminum, chromium, cobalt, zinc, iron, and the like, can be obtained by reacting a salt of the desired heavy metal with the phosphorus sulfide-hydrocarbon reaction product which has been treated with a basic reagent such as above-described.

While the detergent-type additives effectively inhibit the formation of sludge and/or varnish like products in the engine, they do not possess rust and/or corrosion inhibiting properties nor do they possess anti-pitting and anti-wear properties. However, when used in combination with the herein described mixture of the polymerization products of unsaturated fatty acids and with stearic acid, complete engine protection is obtained.

The unsaturated fatty acids which may be polymerized are those natural or synthetic mono-carboxylic acids which generally will have two or more unsaturated linkages. If natural fatty acids are employed they will usually have 16 to 26 carbon atoms, most frequently 18

carbon atoms, but if synthetic unsaturated fatty acids are used they may have a lesser or greater number of carbon atoms. Examples of the natural fatty acids are those such as linoleic, linolenic, ricinoleic (which upon heating forms linoleic acid), linoleidic, elaidololenic, eleostearic, arachidonic, eicosatrienoic, cetoleic, docosatrienoic and the like. The free fatty acids can be polymerized either thermally or with the assistance of catalysts. A method of thermally polymerizing free fatty acids (see U. S. 2,482,761) consists of hydrolyzing a fat or an oil, adding a small portion of water, and heating in a pressure vessel until substantially all of the di- and tri-unsaturated fatty acids present polymerize. The resultant product is then heated at a reduced pressure to distill off vaporizable constituents, leaving behind the polymerized unsaturated fatty acids. The polymerization reaction is carried out at a temperature of about 300° to 360° C. for about three to eight hours at a pressure varying between 75 and 500 p. s. i. g. The polymerization product may consist of monomers, dimers, trimers, and higher polymers of the unsaturated fatty acids. The various fats or oils which may be hydrolyzed to produce the free fatty acids used in the above thermal polymerization are those such as sardine oil, linseed oil, soybean oil, castor oil, peanut oil, palm oil, olive oil, cottonseed oil, sunflower seed oil, and the like.

Another method of preparing the polymerized fatty acids consists of subjecting fats and oils such as have been listed supra (without previous hydrolysis) to a thermal or catalytic polymerization to cause polymerization of the esters of the unsaturated carboxylic acids to the dimers, trimers, and higher polymerization products thereof, followed by hydrolysis to yield the corresponding polymers of the acids. A large source of the polymerized unsaturated fatty acids are those residual acids obtained by methanolysis (see U. S. 2,450,940) of the semi-drying or drying type oils such as castor oil, soybean oil and others listed supra, polymerizing the methyl esters, removing unpolymerized compounds, saponifying the residual esters and freeing polymerized acids therefrom. The products of catalytic polymerization of semi-drying oils such as the  $BF_3$  polymerization products of soybean oil, cottonseed oil, or the like also produce polymers suitable for use in the invention.

It should be understood that while various polymerized unsaturated fatty acids may be used, they do not all provide the same effect, and indeed there may be pronounced differences when used in the composition of this invention. A highly preferred source of the polymerized unsaturated fatty acids is obtained as a by-product still residue in the manufacture of sebacic acid by the dry distillation of castor oil in the presence of sodium hydroxide. A method of obtaining such by-product still residues in the manufacture of sebacic acid is described in U. S. 2,470,849 issued to W. E. Hanson May 24, 1949. The mixture of high molecular weight unsaturated fatty acids comprises monomers, dimers, trimers and higher polymers in the ratio of from about 45% to about 55% of a monomers and dimers fraction having a molecular weight in the range of from about 300 to 600, and from about 45% to about 55% of a trimers and higher polymer fraction having a molecular weight in excess of 600. The fatty acid polymers result in part from a thermal polymerization of fatty acid type constituents of the castor oil, and in part from other reactions, such as the intermolecular esterification, of such acid to form high molecular weight products. The acid mixture, which is mainly a mixture of polymeric long chain polybasic carboxylic acids, is further characterized by the following specifications:

|                    |                  |
|--------------------|------------------|
| Acid No.           | 150 to 164       |
| Saponification No. | 175 to 186       |
| Free fatty acids   | percent 75 to 82 |
| Iodine value       | 44 to 55         |
| Non-saponifiables  | percent 2.5 to 5 |

A fatty acid mixture such as above described is marketed by the W. C. Hardesty Company under the trade name "D-50 Acids," and as "VR-1 Acids" by Rohm and Haas Company.

The polymerization products of the unsaturated fatty acids may have a molecular weight between about 400 and 2000. Those polymers having a molecular weight higher than about 500, and especially those having molecular weights averaging about 800 or higher are particularly preferred for use in this invention. Especially preferred polymerized unsaturated acids are the polymerization products of acids such as linoleic acid having a molecular weight between about 400 and 2000, wherein the polymerization products consist of more than about 40% of the trimer and higher molecular weight polymers of linoleic acid with the remainder consisting primarily of monomers and dimers of linoleic acid. The polymerization products of the unsaturated fatty acids should be used in an amount between about 0.001 and 5.0% in the oil, preferably between about 0.05 to 2.0%, for example about 0.2%. The amount of polymerized fatty acids, as well as the amount of stearic acid used, may be varied depending upon the oil in which it is employed, the materials used in making the cam shaft and valve-lifters, the valve spring pressures and other factors which affect the degree of pitting and wear.

The stearic acid which may be used may be ordinary commercial stearic acid or a purified type of stearic acid. The actual stearic acid content of such compositions may vary from the 45% stearic acid-55% palmitic acid contained in "commercial stearic acid" to the 90% stearic acid which is contained in "commercially pure stearic acid." The stearic acid may be single-, double-, or triple-pressed, preferably the latter. It is contained in the lubricating oil base in amounts between about 0.001 and 5%, preferably between about 0.001 and 2%. As in the case of the polymerized unsaturated fatty acid, the amount of stearic acid may be varied depending upon the intensity of pitting and wear which occur and which is due to factors such as valve-spring pressures, the materials used in the making of the cam-shaft and valve-lifters, additives contained in the oil, etc. A suitable amount of stearic acid is usually about 0.01 to 0.5%. It is to be understood that the amounts of stearic acid as specified herein and in the claims are expressed in terms of the actual stearic acid content of the composition containing stearic acid which is employed. Amine salts such as octadecyl amine salt of stearic acid or metal salts such as zinc stearate may be employed in place of the stearic acid if desired. For example, the aliphatic mono-, di-, or poly-amine salts of stearic acid can be used as well as the alkali, alkaline earth or heavy metal salts of stearic acid. The amine salts may be formed in situ by adding the amine to the oil containing the stearic acid.

The phosphorus- and sulfur-containing detergent-type additive, the polymerization products of the unsaturated fatty acids, and the stearic acid can be added individually to the base motor oil or they can be pre-mixed in the desired proportions and the resultant mixed product added to the base oil. For example, from about 1 to 25% of the polymerized acids, from about 1 to 25% of stearic acid and from about 98 to about 50% of the detergent-type additive can be pre-mixed at a temperature of about 70° to 150° F. and the mixture then added to the base oil. If desired, concentrates of a suitable lubricating oil base containing 10 to about 50% or more of the herein described mixture of polymerized unsaturated fatty acids, stearic acid, and the phosphorus-, sulfur-containing detergent additive may be used for blending with other hydrocarbon lubricating oils in the proportions desired for the particular conditions of use to provide a finished product containing the amounts of the individual constituents previously indicated to be useful. The lubricating oil may also contain other additives such as V. I.

improvers, bearing corrosion inhibitors, rust inhibitors and the like.

A number of performance tests for evaluating the ability of the lubricating oil to inhibit pitting and/or wear as well as its ability to prevent rusting of the hydraulic valve-lifters were made. The tests made to determine the anti-pitting and anti-wear properties of the oil is known as the L-S-5 test established by the General Motors Research Division. The test is made on a 1953 Chevrolet power glide engine equipped with chilled iron lifters, forged steel cams, steel rocker arm shafts, malleable iron rocker arms and operating at 3150 R. P. M. with a load of 30 brake horsepower, an oil sump temperature of 255° F., and a water outlet temperature of 200° F. 5 Dual valve springs are installed to give an assembled static valve spring load of 240 pounds at 0.330 inch valve opening. The test is continued for 24 hours at the end of which the cam followers are inspected for pitting and over-all wear. The effectiveness of the additives for 10 preventing pitting of the cam followers is shown in the table which follows. In this table each sample consisted of an SAE 10W-30 oil containing 3.3% of a barium-containing neutralized reaction product of  $P_2S_5$  and a polybutene of about 1000 molecular weight, 0.75% of a 15 sulfurized dipentene (35% sulfur), and 10 p. p. m. silicone polymer anti-foam agent. Various additives having anti-pitting and anti-wear properties were added to different samples of the oil containing the barium salt, sulfurized dipentene and silicone polymer. The results 20 show:

#### L-S-5 engine tests

| Sample No. | Anti-Pitting and Anti-Wear Additive | Concen-tration, Wt. Per-cent | Lifters Pitted | Rocker Arm Seizure |
|------------|-------------------------------------|------------------------------|----------------|--------------------|
| 35         | None                                |                              | 10             | Severe.            |
| 1.         | D-50 Acid                           | 0.25                         | 3              | Do.                |
| 2.         | D-50 Acid                           | 0.16                         | none           | Moderate.          |
| 3.         | Stearic Acid                        | 0.05                         |                |                    |
| 4.         | D-50 Acid                           | 0.16                         | none           | Do.                |
| 5.         | Amine Stearate                      | 0.20                         | none           | Do.                |
|            | D-50 Acid                           | 0.16                         |                |                    |
|            | Zinc Stearate                       | 0.12                         |                |                    |

<sup>1</sup> Octadecylamine salt of stearic acid.

Sample 1 shows that when no anti-pitting-anti-wear additive is added to the oil, 10 of the 12 cam follower surfaces of the hydraulic valve lifters become pitted. Sample 2 shows that although the D-50 acid (inspections and method of manufacture of which have been detailed previously) is somewhat effective for reducing the number of pitted cam-followers, it does not eliminate the problem of pitting and wear completely. Samples 3, 4, and 5 show that when stearic acid (triple pressed) or its salts such as the octadecyl amine salt of stearic acid or zinc stearate are added to the oil containing the phosphorus- and sulfur-containing detergent-type additive and the polymerized unsaturated fatty acids, there is no pitting at all of the cam follower surfaces.

An additional series of samples were evaluated to determine the ability of various additives to prevent rusting of the hydraulic valve-lifters. The test employed is called the modified Indiana hydraulic valve lifter rust test. This test is carried out in a Chevrolet Powerglide engine operating at 2500 R. P. M. and a load of 45 B. H. P. with an oil temperature of 120° F. and a water temperature of 85-95° F. The test engine is operated at these conditions for 20 hours with a 4 hour running and 4 hour off cycle. At the end of 20 hours the dipstick, rocker arm shaft and valve lifters are inspected for rust. Valve lifters free of rust are rated 10 and badly rusted lifters are rated 1.

The effectiveness of the various additives for preventing rusting and/or corrosion is in the table which follows. In this table each sample consisted of an SAE

SW-20 oil containing 3.3% of a barium-containing neutralized reaction product of  $P_2S_5$  and a polybutene of about 1000 molecular weight, 0.75% of a sulfurized dipentene (35% sulfur), and 10 p. p. m. silicone polymer anti-foam agent. Various additives were added to the oil containing the above ingredients. The results obtained were:

*Modified Indiana hydraulic valve lifter rust test*

| Sam-<br>ple | Additive       | Amount | Engine Ratings (Rust)        |               |                  |
|-------------|----------------|--------|------------------------------|---------------|------------------|
|             |                |        | Dipstick                     | Rocker<br>Arm | Valve<br>Lifters |
| 1           | none           |        | Test stopped, excessive rust |               |                  |
| 6           | Stearic Acid   | 0.20   | Moderate                     | Slight        | 6.0              |
| 7           | Amine Stearate | 0.40   | do                           | do            | 7.0              |
| 8           | D-50 Acid      | 0.16   |                              | Moderate      |                  |
|             | Stearic Acid   | 0.10   | Slight                       |               | 9.5              |

When sample 1 was tested the oil containing the detergent additive caused such severe rusting as to require termination of the test before its normal time. Sample 6 shows that the addition of stearic acid (triple pressed) reduced the amount of rusting. Similarly sample 7 which contained the octadecyl amine salt of stearic acid (triple pressed) reduced the amount of rusting. Evaluation of sample 8 which contained both the polymerized unsaturated fatty acid and stearic acid (triple pressed) showed that the oil containing both such ingredients in addition to the detergent additive reduced rusting of the valve-lifters to a negligible level.

While the present invention has been described by the use of our additives in petroleum lubricating oils, other lubricating oil bases can be employed such as hydrocarbon oils, natural or synthetic such as those obtained by the polymerization of olefines, as well as synthetic lubricating oils of the alkylene oxide type, for example "Ucon Oils" marketed by Carbide and Carbon Corporation, and the polycarboxylic acid ester type oils such as the oil-soluble esters of adipic acid, sebacic acid, azelaic acid, etc.

Unless otherwise stated, the percentages stated herein and in the claims are weight percentages.

Although the present invention has been described with reference to specific preferred embodiments thereof, the invention is not to be considered as limited thereto but

includes within its scope such modifications and variations as come within the spirit of the appended claims.

We claim:

1. A lubricating oil composition having improved valve lifter anti-pitting and anti-wear properties comprising a major proportion of a lubricating mineral oil base, between about 0.002 and 10% of a phosphorus sulfide-hydrocarbon reaction product which has been neutralized with a basic reagent between about 0.001 and 5% of the polymerization products of those unsaturated fatty acids which have between 16 and 26 carbon atoms per molecule, said polymerization products having a molecular weight between about 400 and 2000, and between about 0.001 and 5% of at least one saturated fatty acid compound selected from the class consisting of stearic acid and the salts thereof.
2. The composition of claim 1 wherein the basic reagent is an alkaline earth metal compound.
3. The composition of claim 1 wherein the saturated fatty acid compound is stearic acid.
4. The composition of claim 1 in which the unsaturated fatty acid is linoleic acid.
5. The composition of claim 1 wherein the polymerization products of the unsaturated fatty acids consist of more than about 40% of the trimer and higher molecular weight polymers, the remainder being essentially monomers and dimers of the unsaturated fatty acids.
6. A lubricating oil composition having improved valve lifter anti-pitting and anti-wear properties comprising a major proportion of a lubricating mineral oil base, between about 0.002 and 10% of a phosphorus sulfide-olefin polymer reaction product which has been neutralized with a basic barium compound, between about 0.05 and 2% of the polymerization products of linoleic acid having a molecular weight between about 400 and 2000, said polymerization products consisting of more than about 40% of the trimer and higher molecular weight polymers of linoleic acid and the remainder being essentially monomers and dimers of linoleic acid, and between about 0.001 and 2% of stearic acid.

*References Cited in the file of this patent*

*UNITED STATES PATENTS*

- |    |           |           |               |
|----|-----------|-----------|---------------|
| 45 | 2,281,676 | Cook      | May 5, 1942   |
|    | 2,316,090 | Kelso     | Apr. 6, 1943  |
|    | 2,631,979 | McDermott | Nov. 17, 1953 |